

# United States Patent [19]

Ohno et al.

[11] Patent Number: 4,554,242

[45] Date of Patent: Nov. 19, 1985

[54] METHOD FOR PROCESSING COLOR  
PHOTOGRAPHIC LIGHT-SENSITIVE  
MATERIAL

[75] Inventors: Shigeru Ohno; Shinzo Kishimoto;  
Morio Yagihara, all of Kanagawa,  
Japan

[73] Assignee: Fuji Photo Film Co., Ltd., Kanagawa,  
Japan

[21] Appl. No.: 690,068

[22] Filed: Jan. 9, 1985

[30] Foreign Application Priority Data

Jan. 12, 1984 [JP] Japan ..... 59-4018

[51] Int. Cl.<sup>4</sup> ..... G03C 7/00

[52] U.S. Cl. ..... 430/393; 430/429;  
430/430; 430/460; 430/461

[58] Field of Search ..... 430/393, 429, 430, 460,  
430/461

[56] References Cited

U.S. PATENT DOCUMENTS

3,617,283 11/1971 Ohi et al. ..... 430/393  
3,645,738 2/1972 Willems et al. ..... 430/429  
3,820,997 6/1974 Shirasu et al. ..... 430/393  
4,144,068 3/1979 Ishibashi et al. ..... 430/393  
4,292,401 9/1981 Itoh et al. ..... 430/461

Primary Examiner—J. Travis Brown

Attorney, Agent, or Firm—Sughrue, Mion, Zinn,  
Macpeak & Seas

## ABSTRACT

A method for processing a color photographic light-sensitive material by subjecting an exposed silver halide color photographic light-sensitive material to color development, then to bleaching and fixing or then to bleach-fixing, which method comprises using a ferric ion complex salt as a bleaching agent in the bleaching or bleach-fixing and incorporating at least one compound represented by general formula (I) described below or a tautomer thereof:



wherein all the symbols are defined in the appended claims, in a bleaching bath or bleach-fixing bath or in a prebath of the bleach-fixing bath. The method of the present invention does not produce poisonous materials which are harmful to the environment and provides an excellent high speed bleaching process without harming other photographic properties.

20 Claims, No Drawings

## METHOD FOR PROCESSING COLOR PHOTOGRAPHIC LIGHT-SENSITIVE MATERIAL

### FIELD OF THE INVENTION

The present invention relates to a method for processing an exposed silver halide color photographic light-sensitive material (hereinafter referred to as a color light-sensitive material) which comprises developing, bleaching, and fixing (hereinafter referred to as a color photographic processing method), and, more particularly, to an improved bleaching process which accelerates the bleaching function, thus shortening the processing time while providing sufficient bleaching, thus providing a color photographic image of good image quality.

### BACKGROUND OF THE INVENTION

The fundamental steps of processing color light-sensitive materials generally include a color developing and a silver removal. Thus, an exposed silver halide color photographic light-sensitive material is introduced into a color developing step, where silver halide is reduced with a color developing agent to produce silver and the oxidized color developing agent in turn reacts with a color former to yield a dye image. Subsequently, the color photographic material is introduced into a silver removal step, where silver produced in the preceding step is oxidized with an oxidizing agent (usually called a bleaching agent), and dissolved away with a silver ion complexing agent usually called a fixing agent. Therefore, only a dye image is formed in the thus processed photographic material. In addition to the above described two fundamental steps of color development and silver removal, actual development processing involves auxiliary steps for maintaining the photographic and physical quality of the resulting image or for improving the preservability of the image. For example, there are illustrated a hardening bath for preventing a light-sensitive layer from being excessively softened during photographic processing, a stopping bath for effectively stopping the developing reaction, an image stabilizing bath for stabilizing the image, and a layer removing bath for removing the backing layer on the support.

The above described silver removal may be conducted in two ways: one way uses two steps employing a bleaching bath and a fixing bath; and the other way is more simple and is conducted in one step employing a bleach-fixing (or blixing) bath containing both a bleaching agent and a fixing agent for the purpose of accelerating the processing and labor elimination.

Ferricyanide and ferric chloride, heretofore used as bleaching agents, are good bleaching agents due to their high oxidizing power. However, a bleaching solution or bleach-fixing solution containing ferricyanide can release poisonous cyanide by photolysis causing environmental pollution. Accordingly, waste processing solutions thereof must be rendered harmless in view of environmental pollution. A bleaching solution containing ferric chloride as a bleaching agent is not desirable because materials of vessels in which the solution is retained are liable to be corroded due to the extremely low pH and high oxidizing power of the solution. In addition, iron hydroxide is precipitated in an emulsion layer during water-washing after a bleaching step using ferric chloride, resulting in staining.

On the other hand, potassium dichromate, quinones, copper salts, etc., which have been used as bleaching agents have weak oxidizing power and are difficult to handle.

5 In recent years, bleach processing using a ferric ion complex salt (e.g., aminopolycarboxylic acidferric ion complex salt, particularly iron (III) ethylenediaminetetraacetate complex salt) as a major bleach bath component has mainly been employed in processing color photographic light-sensitive materials in view of the acceleration and simplification of the bleaching provided and the need to prevent environmental pollution.

However, ferric ion complex salts have a comparatively low oxidizing power and, therefore, have insufficient bleaching power. A bleaching or bleach-fixing solution containing such a complex salt as a bleaching agent can attain some desirable objects when bleaching or bleach-fixing a low speed silver halide color photographic light-sensitive material containing, for example, a silver chlorobromide emulsion as a major component. However, such a solution fails to fully remove silver due to insufficient bleaching power or requires a long time to bleach when processing a high speed, spectrally sensitized silver halide color photographic light-sensitive material containing a silver chlorobromoiode emulsion or a silver iodobromide emulsion as a major component, particularly color reversal light-sensitive materials for photographing or color negative light-sensitive materials for photographing comprising an emulsion containing a larger amount of silver.

As described above, bleaching agents which do not cause environmental pollution or corrode vessels and apparatus have only a weak bleaching power. Hence, it is requested to enhance the bleaching power of a bleaching or bleach-fixing solution containing a weak bleaching agent, particularly a ferric ion complex salt.

In order to raise the bleaching power of a bleaching or bleach-fixing solution containing a ferric ion complex salt such as iron (III) ethylenediaminetetraacetate as a bleaching agent, it has been proposed to add various bleach accelerating agents to the processing bath.

Examples of such bleach accelerating agents include 5-membered heterocyclic mercapto compounds as described in British Pat. No. 1,138,842. However, these compounds do not necessarily have sufficient bleach accelerating effects when they are added to a bleaching solution or a prebath thereof. Also, only insufficient bleach accelerating effects are obtained when they are added to a bleach-fixing solution or a prebath thereof. Further, in the latter case they react with silver ions present in the bleach-fixing solution to form precipitate which creates many troubles. For example, the precipitate chokes up filters of a circulation system in an automatic processing machine and it adheres on photographic light-sensitive materials, resulting in stain formation.

A processing method is also known wherein a 5-membered heterocyclic compound containing two or three nitrogen atoms as ring constituting members and having at least one mercapto group is added to a bath just before a bath of the bleaching processing as described in Japanese Patent Application (OPI) No. 52534/79 (the term "OPI" as used herein refers to a "published unexamined Japanese patent application"). However, when these compounds are directly added to a bleaching solution or a bleach-fixing solution, sufficient bleach accelerating effects cannot be obtained. In

addition, they lack stability in the processing solution and cannot endure use for a long period of time.

Moreover, thiourea derivatives as described in Japanese Patent Publication No. 8506/70 (corresponding to U.S. Pat. No. 3,617,283) and U.S. Pat. No. 3,706,561, and selenourea derivatives as described in Japanese Patent Application (OPI) No. 280/71 (corresponding to U.S. Pat. No. 3,701,662) are known as bleach accelerating agents. However, many of these bleach accelerating agents do not always show a satisfactory bleach accelerating effect, or some of them lack stability in the processing solution although they have a good bleach accelerating effect. Therefore, they provide a processing solution having only a short effective life or which cannot be stored for a long time.

Furthermore, heterocyclic alkylmercaptan derivatives as described in Japanese Patent Application (OPI) No. 32736/78, and aminoalkylmercaptan derivatives as described in U.S. Pat. No. 3,893,858 are known as bleach accelerating agents. However, these bleach accelerating agents do not always show a satisfactory bleach accelerating effect, or they retard fixing even although they can accelerate bleaching. Therefore, a long period of time is necessary for silver removal processing.

#### SUMMARY OF THE INVENTION

An object of the present invention is to provide a method for processing a color photographic material, which does not release extremely poisonous materials, which meets the requirement of preventing environmental pollution and which has excellent bleaching speed.

Another object of the present invention is to provide a method involving a bleaching or bleach-fixing step in which enhanced bleaching power is attained without deteriorating other photographic properties using a bleaching agent having a weak bleaching power, in particular a ferric ion complex salt.

A further object of the present invention is to provide a bleaching process which uses a bleaching or bleach-fixing solution showing increased bleaching speed and having good stability.

A still further object of the present invention is to provide a method which can rapidly bleach or bleach-fix a color photographic light-sensitive material having a photographic sensitivity.

Other objects of the present invention will become apparent from the following description and Examples.

These objects of the present invention are reached by a method for processing a color photographic light-sensitive material comprising subjecting an exposed silver halide color photographic light-sensitive material to color development then to bleaching and to fixing or then to bleach-fixing, which process comprises using a ferric ion complex salt as a bleaching agent in the bleaching or bleach-fixing and incorporating at least one compound represented by general formula (I) described below or a tautomer thereof in a bleaching bath or a bleach-fixing bath or in a prebath of the bleach-fixing bath.



wherein X represents N or C-R; R, R<sup>1</sup>, R<sup>2</sup> and R<sup>3</sup>, which may be the same or different, each represents a hydrogen atom, a halogen atom, an amino group, a hydroxyl group, a carboxyl group, a sulfo group or an alkyl group which includes an unsubstituted alkyl group and a substituted alkyl group; R<sup>4</sup> and R<sup>5</sup>, which may be the same or different, each represents a hydrogen atom, an alkyl group which includes an unsubstituted alkyl group and a substituted alkyl group, or an acyl group, or R<sup>4</sup> and R<sup>5</sup> may be bonded to each other to form a ring, provided that both R<sup>4</sup> and R<sup>5</sup> do not represent a hydrogen atom at the same time; and n represents an integer of 0 to 5.

#### DETAILED DESCRIPTION OF THE INVENTION

The compounds represented by general formula (I) are described in more detail below.

In general formula (I), the halogen atom represented by R, R<sup>1</sup>, R<sup>2</sup> or R<sup>3</sup> include a chlorine atom, a bromine atom, etc.

The alkyl group represented by R, R<sup>1</sup>, R<sup>2</sup>, R<sup>3</sup>, R<sup>4</sup> or R<sup>5</sup> is preferably an unsubstituted or substituted one having from 1 to 5 carbon atoms in the alkyl moiety (for example, a methyl group, an ethyl group, a propyl group, etc.). Examples of substituents for the substituted alkyl group include a halogen atom, a hydroxyl group, an alkoxy group (for example, a methoxy group, an ethoxy group, etc.), a sulfonyl group (for example, a methanesulfonyl group, an ethanesulfonyl group, etc.), a carbamoyl group, a sulfamoyl group, a carboxyl group, a sulfo group, an amino group (for example, an unsubstituted amino group, a dimethylamino group, etc.), an amido group (for example, an acetylamino group, etc.) or a sulfonamido group (for example, a methanesulfonylamino group, etc.), etc.

The ring formed by bonding R<sup>4</sup> and R<sup>5</sup> includes a pyrrole ring, an imidazole ring, a pyrazole ring, a piperidine ring, a morpholine ring, etc.

The acyl group represented by R<sup>4</sup> or R<sup>5</sup> is preferably one having 3 or less carbon atoms. Particularly, an acetyl group is preferred.

The tautomer of the compound represented by general formula (I) has the following general formula:



wherein all the symbols are the same as described above.

According to the present invention, the bleach accelerating agents which have a sufficient bleach accelerating effect and good stability in the processing solution can be provided by introducing an alkyl group or an

acyl group into at least one of  $R^4$  and  $R^5$  in general formula (I).

Specific examples of the compounds represented by general formula (I) are set forth below, but the present invention should not be construed as being limited thereto.



(1) 10



(2) 15



(3) 25



(4) 30



(5) 35



(6) 40



(7) 45



(8) 50



(9) 55



(10) 60

65

-continued



(11)



(12)



(13)



(14)



(15)



(16)



(17)



(18)



(19)



(20)



(21)



The compounds represented by general formula (I) used in the present invention can be synthesized by the methods as described in A. Whohl and W. Marckwald, *Ber.*, Vol. 22, page 568 (1889), M. Freund, *Ber.*, Vol. 29, page 2483 (1896), A. P. T. Easson et al., *J. Chem. Soc.*, Vol. 1932, page 1806, R. G. Jones et al., *J. Am. Chem. Soc.*, Vol. 71, page 4000 (1949), etc. Further they can be synthesized with reference to the typical Synthesis Examples as described in the following.

In the Synthesis Examples and Examples described below, unless otherwise indicated, all parts, percents, ratios and the like are by weight.

#### SYNTHESIS EXAMPLE 1

##### Synthesis of Compound (3)

13.3 g of aminoacetaldehyde diethylacetal was dissolved in 100 ml of carbon tetrachloride and to the solution was gradually added 13 g of 2-dimethylaminethyl isothiocyanate under cooling with ice. The mixture was stirred for 2 hours at room temperature and then the solvent was distilled off under reduced pressure. To the residue thus obtained was added 110 ml of a 35% sulfuric acid under cooling with ice and then the mixture was refluxed by heating for 3 hours. The reaction solution was neutralized with a 30% aqueous solution of sodium hydroxide and extracted with chloroform. The organic layer was dried with anhydrous sodium sulfate, the solvent was distilled off under reduced pressure and the residue thus obtained was recrystallized from ethyl acetate. Yield: 6.8 g. Melting Point: 130° to 131° C.

#### SYNTHESIS EXAMPLE 2

##### Synthesis of Compound (6)

13.3 g of aminoacetaldehyde diethylacetal was dissolved in 100 ml of carbon tetrachloride and to the solution was added dropwise 14.4 g of 3-dimethylaminopropyl isothiocyanate under cooling with ice. The mixture was stirred at room temperature for 2 hours and then the solvent was distilled off under reduced pressure. To the residue thus obtained was added 110 ml of a 35% sulfuric acid under cooling with ice and then the mixture was refluxed by heating for 3 hours.

8

The reaction solution was neutralized with a 30% aqueous solution of sodium hydroxide and extracted with chloroform. The organic layer was dried with anhydrous sodium sulfate, the solvent was distilled off under reduced pressure and the residue thus obtained was recrystallized from ethyl acetate. Yield: 9.6 g. Melting Point: 120° to 121° C.

#### SYNTHESIS EXAMPLE 3

##### Synthesis of Compound (9)

13.3 g of aminoacetaldehyde diethylacetal was dissolved in 100 ml of carbon tetrachloride and to the solution was added dropwise 15.8 g of 2-diethylaminethyl isothiocyanate under cooling with ice. The mixture was stirred at room temperature for 2.5 hours and then the solvent was distilled off under reduced pressure. To the residue thus obtained was added 110 ml of a 35% sulfuric acid under cooling with ice and then the mixture was refluxed by heating for 3 hours. The reaction solution was neutralized with a 30% aqueous solution of sodium hydroxide and extracted with chloroform. The organic layer was dried with anhydrous sodium sulfate, the solvent was distilled off under reduced pressure and the residue thus obtained was recrystallized from ethyl acetate. Yield: 6.4 g. Melting Point: 101° to 102° C.

#### SYNTHESIS EXAMPLE 4

##### Synthesis of Compound (13)

13.3 g of aminoacetaldehyde diethylacetal was dissolved in 100 ml of carbon tetrachloride and to the solution was added dropwise 17.2 g of 2-(N-morpholino)-ethyl isothiocyanate under cooling with ice. The mixture was stirred at room temperature for 2.5 hours and then the solvent was distilled off under reduced pressure. To the residue thus obtained was added 110 ml of a 35% sulfuric acid solution under cooling with ice and then the mixture was refluxed by heating for 4 hours. The reaction solution was neutralized with a 30% aqueous solution of sodium hydroxide and extracted with chloroform. The organic layer was dried with anhydrous sodium sulfate, the solvent was distilled off under reduced pressure and the residue thus obtained was recrystallized from isopropyl alcohol. Yield: 7.5 g. Melting Point: 154° to 156° C.

#### SYNTHESIS EXAMPLE 5

##### Synthesis of Compound (15)

To a solution of 7.5 ml of hydrazine hydrate and 30 ml of ethanol was gradually added 6.5 g of 2-dimethylaminooethyl isothiocyanate under cooling with ice and then the mixture was stirred for 3 hours. The reaction solution was added to 100 ml of water and extracted with chloroform. The organic layer was washed with a saturated aqueous solution of sodium chloride and then the solvent was distilled off under reduced pressure. To 7.2 g of the residue thus obtained was added 36 ml of formic acid and the mixture was refluxed by heating for 8 hours. The reaction solution was concentrated under reduced pressure, and the residue thus obtained was neutralized with a 5% aqueous solution of sodium hydroxide, purified by column chromatography (stationary phase: alumina; spreading solvent: ethyl acetate/methanol) and recrystallized from ethyl acetate/n-hexane. Yield: 3.8 g. Melting Point: 103° to 104° C.

## SYNTHESIS EXAMPLE 6

## Synthesis of Compound (18)

To a solution of 7.5 ml of hydrazine hydrate and 30 ml of ethanol was added dropwise 7.2 g of 3-dimethylaminopropyl isothiocyanate under cooling with ice and then the mixture was stirred for 3 hours. The reaction solution was added to 100 ml of water and extracted with diethyl ether. The ether layer was washed with a saturated aqueous solution of sodium chloride and then the solvent was distilled off under reduced pressure. To 7.8 g of the residue thus obtained was added 40 ml of formic acid and the mixture was refluxed by heating for 8 hours. The reaction solution was concentrated under reduced pressure, and the residue thus obtained was neutralized with a 5% aqueous solution of sodium hydroxide, purified by column chromatography (stationary phase: alumina; spreading solvent: ethyl acetate/methanol) and recrystallized from isopropyl alcohol. Yield: 4.5 g. Melting Point: 161° to 163° C.

## SYNTHESIS EXAMPLE 7

## Synthesis of Compound (22)

To a solution of 7.5 ml of hydrazine hydrate and 30 ml of ethanol was added dropwise 8.6 g of 2-(N-morpholino)ethyl isothiocyanate under cooling with ice and then the mixture was stirred for 2 hours. The precipitate thus formed was collected by filtration to obtain 9.5 g of the crystals. To the crystals was added 50 ml of formic acid and the mixture was refluxed by heating for 8 hours. The reaction solution was concentrated under reduced pressure, and the residue thus obtained was neutralized with a 5% aqueous solution of sodium hydroxide, purified by column chromatography (stationary phase: alumina; spreading solvent: ethyl acetate/methanol) and recrystallized from chloroform. Yield: 4.9 g. Melting Point: 146° to 147° C.

The compounds of the above described general formula (I) used in the present invention as a bleach accelerating agent can be incorporated directly into a bleaching bath or a bleach-fixing bath, whereby a processing bath which is stable for a long period of time and has a satisfactory bleaching function can be provided. Further, the compound may be incorporated into a prebath of a bleach-fixing bath, or may be incorporated into both a bleach-fixing bath and a prebath thereof.

The amount of the compound according to the present invention added to these solutions varies depending upon the kind of processing solution, kind of photographic material to be processed, processing temperature, time necessary for conducting intended processing, etc. However, an amount of about  $1 \times 10^{-5}$  to about 1 mol per liter of a processing solution is suitable, with  $1 \times 10^{-4}$  to  $1 \times 10^{-1}$  mol being preferable. In general, however, when the amount added is small, there results a small bleach accelerating effect, whereas when the amount is more than is necessary, a precipitate may be formed which stains processed materials. Therefore, the best range is properly determined with consideration for individual cases.

The compound according to the present invention is generally added to a processing solution by previously dissolving it in water, an alkali (e.g., sodium hydroxide), an organic acid (e.g., acetic acid or propionic acid), or the like. If necessary, an organic solvent (e.g., methyl alcohol or ethyl alcohol) may be used for dissolving the

compound without adversely affecting its bleach accelerating effect.

When incorporating the compound according to the present invention into a prebath of a bleach-fixing solution, the amount to be added is suitably from about  $1 \times 10^{-5}$  to about 1 mol per liter of the prebath and preferably from  $1 \times 10^{-4}$  to  $1 \times 10^{-1}$  mol per liter of the prebath. The prebath may have various compositions. A prebath having the simplest composition is an aqueous solution prepared by merely dissolving the compound according to the present invention in water. Aqueous solutions properly containing acids such as acetic acid, boric acid, etc., alkalis such as sodium hydroxide, etc., or salts such as sodium acetate, sodium thiosulfate, sodium borate, sodium carbonate, sodium bicarbonate, etc., are also usable as prebaths with advantage. Prebaths having any pH may be used with satisfactory effects in the present invention. However, too high of a pH may generate stain, and hence prebaths having a pH of 9 or less are generally preferable. The prebath may further contain, if necessary, precipitation preventing agents comprising various chelate compounds; hardeners comprising various compounds including alums or aldehydes; pH buffers; fixing agents for halides; antioxidants such as sulfites, hydroxylamine, hydrazine, etc.; swelling preventing agents such as sodium sulfate, magnesium sulfate, etc.; surfactants; and the like.

Between the prebath and the bleach-fixing bath may be provided, for example, a water-washing step, stopping step, stop-fixing step, or the like. In such cases, the addition of the compound according to the present invention to the prebath will also bring about the same bleach accelerating effect. However, where the compound according to the present invention is incorporated only in the prebath, the prebath is preferably provided immediately before a bleach-fixing bath.

In the bleaching solution or bleach-fixing solution of the present invention, a weak bleaching agent is used. A ferric ion complex, one of the bleaching agents, is a complex of ferric ion and a chelating agent such as an aminopolycarboxylic acid, an aminopolyphosphonic acid or the salt thereof. Aminopolycarboxylic acid salts or aminopolyphosphonic acid salts are alkali metal salts, ammonium salts or water-soluble amine salts of aminopolycarboxylic acids or aminopolyphosphonic acids. The alkali metals include sodium, potassium, lithium, etc., and water-soluble amines include alkylamines (e.g., methylamine, diethylamine, triethylamine, butylamine, etc.), alicyclic amines (e.g., cyclohexylamine), arylamines (e.g., aniline, m-toluidine, etc.), and heterocyclic amines (e.g., pyridine, morpholine, piperidine, etc.).

Typical examples of these chelating agents, i.e., aminopolycarboxylic acids, aminopolyphosphonic acids, and the salts thereof are:

Ethylenediaminetetraacetic acid;  
Disodium ethylenediaminetetraacetate;  
Diammonium ethylenediaminetetraacetate;  
Tetra(trimethylammonium)ethylenediaminetetraacetate;  
Tetrapotassium ethylenediaminetetraacetate;  
Tetrasodium ethylenediaminetetraacetate;  
Trisodium ethylenediaminetetraacetate;  
Diethylenetriaminepentaacetic acid;  
Pentasodium diethylenetriaminepentaacetate;  
Ethylenediamine-N-( $\beta$ -oxyethyl)-N,N',N'-triacetic acid;

Trisodium ethylenediamine-N-( $\beta$ -oxyethyl)-N,N',N'-triacetate;  
 Triammonium ethylenediamine-N-( $\beta$ -oxyethyl)-N,N',N'-triacetate;  
 Propylenediaminetetraacetic acid;  
 Disodium propylenediaminetetraacetate;  
 Nitrilotriacetic acid;  
 Trisodium nitrilotriacetate;  
 Cyclohexanediaminetetraacetic acid;  
 Disodium cyclohexanediaminetetraacetate;  
 Iminodiacetic acid;  
 Dihydroxyethylglycine;  
 Ethyl ether diaminetetraacetic acid;  
 Glycol ether diaminetetraacetic acid;  
 Ethylenediaminetetrapropionic acid;  
 Phenylenediaminetetraacetic acid;  
 1,3-Diaminopropanol-N,N,N',N'-tetramethylene-phosphonic acid;  
 Ethylenediamine-N,N,N',N'-tetramethylenephosphonic acid;  
 1,3-Propylenediamine-N,N,N',N'-tetramethylene-phosphonic acid; etc.

The present invention is not limited to the above illustrated chelating agents.

The ferric ion complex salts may be used in the form of a complex salt per se or may be formed in situ in solution by using a ferric salt (e.g., ferric sulfate, ferric chloride, ferric nitrate, ferric ammonium sulfate or ferric phosphate, etc.) and a chelating agent (e.g., aminopolycarboxylic acid, aminopolyphosphonic acid or phosphonocarboxylic acid, etc.). When they are used in the form of a complex salt, they may be used alone or as a combination of two or more. On the other hand, where a complex is formed in situ in solution by using a ferric salt and a chelating agent, one, two or more ferric salts may be used. Further, one, two or more chelating agents may also be used. In every case, a chelating agent may be used in an excess amount of being necessary for forming a ferric ion complex salt.

A bleaching solution or a bleach-fixing solution containing the above-described ferric ion complex may further contain complexes of metals other than iron such as cobalt or copper or hydrogen peroxide. The bleach accelerating agents according to the present invention are, of course, effective for the persulfates, but show particularly remarkable effects on ferric ion complex salts.

The bleaching solution used in the present invention can contain re-halogenating agents such as bromides (e.g., potassium bromide, sodium bromide, ammonium bromide, etc.), chlorides (e.g., potassium chloride, sodium chloride, ammonium chloride, etc.), and the like in addition to the bleaching agents such as ferric ion complex salts, etc., and the above described compounds. Further, additives which have a pH buffering ability such as inorganic acids, organic acids, or the salts thereof which are known to be used in ordinary bleaching solutions (e.g., boric acid, borax, sodium metaborate, acetic acid, sodium acetate, sodium carbonate, potassium carbonate, phosphorous acid, phosphoric acid, sodium phosphate, citric acid, sodium citrate, tartaric acid, etc.) may be added.

The amount of bleaching agent is from about 0.1 to about 2 mols per liter of the bleaching solution, and the pH of the bleaching solution is desirably from about 3.0 to about 8.0, particularly from 4.0 to 7.0, when a ferric ion complex salt is used.

On the other hand, when the compound according to the present invention is employed in a bleach-fixing solution, ordinary fixing agents, i.e., water-soluble silver halide-dissolving agents such as thiosulfates (e.g., sodium thiosulfate, ammonium thiosulfate, ammonium sodium thiosulfate, potassium thiosulfate, etc.); thiocyanates (e.g., sodium thiocyanate, ammonium thiocyanate, potassium thiocyanate, etc.); thioether compounds (e.g., ethylenebisthioglycolic acid, 3,6-dithia-1,8-octanediol, etc.); and thioureas may be used alone or as a combination of two or more. In addition, special bleach-fixing solution comprising a combination of a fixing agent as described in Japanese Patent Application (OPI) No. 155354/80 and 1.7 mol or more of a halide compound such as potassium iodide per liter of the bleach-fixing solution can be used as well.

In the bleach-fixing composition, the ferric ion complex salt is present in an amount of about 0.1 to about 2 mols and the amount of fixing agent is from 0.2 to 4 mols, per liter of the bleach-fixing solution.

A bleach-fixing solution can contain the aforesaid additives to be added to the bleaching solution and preservatives such as sulfites (e.g., sodium sulfite, potassium sulfite, ammonium sulfite, etc.), hydroxylamine, hydrazine, aldehyde-bisulfite adducts (e.g., acetaldehyde-sodium bisulfite adduct), etc. Further, various fluorescent brightening agents, defoaming agents, surfactants, organic solvents (e.g., methanol), and known bleach-fixing accelerating agents (e.g., polyamine compounds as described in Japanese Patent Publication No. 8836/70, thiourea derivatives as described in Japanese Patent Publication No. 8506/70, iodides as described in German Pat. No. 1,127,715, polyethylene oxides as described in German Pat. No. 966,410, nitrogen-containing heterocyclic compounds as described in German Pat. No. 1,290,812, and other thioureas) may be used. The pH of the bleach-fixing solution upon use is usually from 4.0 to 9.0, particularly preferably from 5.0 to 8.0.

The above described bleaching agent or bleaching agent composition can be a bleaching solution for use as is or for use as a replenishing solution and as a preparation for manufacturing a bleaching solution. When two or more liquid preparations are used, the pH of the liquid preparation containing a ferric ion complex salt can be further increased irrespective of the pH range as described above.

Both bleach processing and bleach-fixing processing are preferably conducted at temperatures of about 25° to 45° C. for about 30 seconds to 10 minutes. When prebath processing is employed, it is preferably conducted at temperatures of about 25° to 45° C. for 5 minutes or less and at least 1 second.

Primary aromatic amine color developing agents to be used in the present invention in a color developing solution include a wide range of known developing agents for use in various color photographic processes. The developing agents include aminophenol derivatives and p-phenylenediamine derivatives. These compounds are generally used in the form of salts such as hydrochlorides or sulfates rather than in free form in view of stability advantages. They are generally used in an amount of from about 0.1 g to about 30 g, more preferably from about 1 g to about 15 g, per liter of color developing solution.

The aminophenol type developing agents include, for example, o-aminophenol, p-aminophenol, 5-amino-2-

hydroxytoluene, 2-amino-3-hydroxytoluene, 2-hydroxy-3-amino-1,4-dimethylbenzene, etc.

Particularly useful primary aromatic amine type color developing agents are N,N-dialkyl-p-phenylenediamine compounds where the alkyl group and the phenyl group may or may not be substituted. Of these, particularly useful compounds are N,N-diethyl-p-phenylenediamine hydrochloride, N-methyl-p-phenylenediamine hydrochloride, N,N-dimethyl-p-phenylenediamine hydrochloride, 2-amino-5-(N-ethyl-N-dodecylamino)toluene, N-ethyl-N-β-methanesulfonamidoethyl-3-methyl-4-aminoaniline sulfate, N-ethyl-N-β-hydroxyethylaminoaniline, 4-amino-3-methyl-N,N-diethylaniline, 4-amino-N-(2-methoxyethyl)-N-ethyl-3-methylaniline p-toluenesulfonate, etc.

The alkaline color developing solution used in the present invention can optionally contain, in addition to the above described primary aromatic amine color developing agent, various ingredients usually added to a color developing solution, such as alkali agents (e.g., sodium hydroxide, sodium carbonate, potassium carbonate, etc.), alkali metal sulfites, alkali metal bisulfites, alkali metal thiocyanates, alkali metal halides, benzyl alcohol, water-softening agents, thickening agents, etc. The pH of the color developing solution is usually 7 or above, most generally from about 9 to about 13.

The process of the present invention is applicable to color reversal processing. In the present invention, as a black-and-white developing solution to be used in such processing, a black-and-white first developing solution used for reversal processing of color photographic light-sensitive materials or used for processing black-and-white photographic light-sensitive materials can be used. In addition, various well known additives generally added to a black-and-white developing solution can be incorporated in the solution.

Typical additives include developing agents such as 1-phenyl-3-pyrazolidone, metol, and hydroquinone; preservatives such as sulfites; pH buffering agents comprising an alkali such as sodium hydroxide, sodium carbonate, or potassium carbonate; inorganic or organic inhibitors such as potassium bromide, 2-methylbenzimidazole, methylbenzothiazole, etc.; water-softening agents such as polyphosphoric acid salts; and slight amounts of development restrainers comprising an iodide or a mercapto compound.

Silver halide color photographic light-sensitive materials processed according to the present invention in the presence of the compounds according to the present invention are known color photographic light-sensitive materials. The present invention is particularly advantageous for processing coupler-containing multilayer negative color photographic light-sensitive materials or color print photographic light-sensitive materials or for processing color photographic light-sensitive materials designed to be subjected to reversal color processing. In addition, color X-ray photographic light-sensitive materials, monolayer special color photographic light-sensitive materials, and color photographic light-sensitive materials containing a black-and-white developing agent such as a 3-pyrazolidone as described in U.S. Pat. Nos. 2,751,297 and 3,902,905 and Japanese Patent Application (OPI) Nos. 64339/81, 85748/81 and 85749/81, and a color developing agent precursor as described in U.S. Pat. Nos. 2,478,400, 3,342,597, 3,342,599, 3,719,492 and 4,214,047 and Japanese Patent Application (OPI) No. 135628/78 can be processed according to the pres-

ent invention. Further, the processing may be conducted with a coupler in the developing solution.

In a photographic emulsion layer of a color light-sensitive material used in the present invention, any of silver bromide, silver iodobromide, silver iodochlorobromide, silver chlorobromide, and silver chloride may be used as a silver halide.

During formation or physical ripening of the silver halide grains, cadmium salts, zinc salts, lead salts, thallium salts, iridium salts or complex salts thereof, rhodium salts or complex salts thereof, iron salts or complex salts thereof, etc., may be present.

In the present invention, both negative emulsions forming surface latent images and direct reversal emulsions can be used. Examples of the latter emulsions include emulsions forming internal latent images and previously fogged direct reversal emulsions.

The silver halide emulsions used are preferably chemically sensitized. That is, sulfur sensitization using sulfur-containing compounds capable of reacting with silver ions or active gelatin, reduction sensitization using a reductive substance, and noble metal sensitization using compounds of noble metals such as gold can be employed alone or in combination. Examples of useful sulfur sensitizers include thiosulfates, thioureas, thiazoles, rhodanines, and other compounds. Examples of useful reduction sensitizers include stannous salts, amines, hydrazine derivatives, formamidinesulfonic acids and silane compounds. For noble metal sensitization, complexes of group VIII metals in the Periodic Table such as platinum, iridium, palladium, etc., can be used as well as gold complexes.

The photographic emulsions may be spectrally sensitized with methine dyes or the like. Dyes used include cyanine dyes, merocyanine dyes, complex cyanine dyes, complex merocyanine dyes, holopolar cyanine dyes, hemicyanine dyes, styryl dyes and hemioxonol dyes. Particularly useful dyes are those belonging to cyanine dyes, merocyanine dyes and complex merocyanine dyes.

The light-sensitive material according to the present invention may contain a polyalkylene oxide or its ether, ester or amine derivative thereof, a thioether compound, a thiomorpholine, a quaternary ammonium salt compound, a urethane derivative, a urea derivative, an imidazole derivative, a 3-pyrazolidone, etc., for the purpose of increasing sensitivity or contrast or for accelerating development.

As binders for photographic emulsion layers or other layers, gelatin is advantageously employed, but other hydrophilic colloids may also be used.

Various compounds may be incorporated in the light-sensitive material according to the present invention as antifoggants or stabilizers. That is, many compounds known as antifoggants or stabilizers such as azoles (e.g., benzothiazolium salts, nitroindazoles, triazoles, benzotriazoles, benzimidazoles (particularly, nitro- or halogen-substituted derivatives), etc.); heterocyclic mercapto compounds (e.g., mercaptothiazoles, mercapto-benzothiazoles, mercaptobenzimidazoles, mercaptodiimidazoles, mercaptotetrazoles (e.g., 1-phenyl-5-mercaptopentetrazole), and mercaptopyrimidines); the above described heterocyclic mercapto compounds having a water-soluble group such as a carboxyl group or a sulfo group; thioketo compounds (e.g., oxazolinethione); azaindenes (e.g., tetraazaindenes (particularly 4-hydroxy-substituted (1,3,3a,7)tetraazaindenes)); ben-

zenethiosulfonic acids; benzenesulfinic acids; etc., can be added.

The photographic light-sensitive material according to the present invention may contain an organic or inorganic hardener in its photographic emulsion layers or other layers. For example, chromium salts, aldehydes, active vinyl compounds (e.g., 1,3,5-triacryloyl-hexahydro-s-triazine, 1,3-vinylsulfonyl-2-propanol, etc.), active halogen compounds (e.g., 2,4-dichloro-6-hydroxy-s-triazine, etc.), mucohalogenetic acids, etc., can be used alone or in combination.

The photographic light-sensitive material according to the present invention may contain in its photographic emulsion layers or other layers various surfactants for various purposes such as improvement of coating properties, antistatic properties, slipping properties, emulsion dispersibility, anti-adhesion properties, and photographic properties (for example, development acceleration, increase in contrast, sensitization, etc.).

The light-sensitive material according to the present invention contains in its photographic emulsion layers color forming couplers, that is, compounds capable of forming color by oxidative coupling with an aromatic primary amine developing agent (for example, a phenylenediamine derivative or an aminophenol derivative) in color development processing. For example, magenta couplers include 5-pyrazolone couplers, pyrazolobenzimidazole couplers, cyanoacetylcoumarone couplers, open chain acyl-acetonitrile couplers, etc., yellow couplers include acylacetamide couplers (e.g., benzoylacetanilides, pivaloylacetanilides, etc.), and cyan couplers include naphthol couplers, phenol couplers, etc. Of these couplers, nondiffusible couplers having a hydrophobic group called a ballast group are desirable. The couplers may be of either 4-equivalent type or 2-equivalent type to silver ions. Colored couplers having a color correcting effect or couplers capable of releasing a development inhibitor upon development (so-called DIR couplers) may also be used. In addition to DIR couplers, non-color forming DIR coupling compounds capable of forming a colorless coupling reaction product and releasing a development inhibitor and DIR redox compounds may also be incorporated.

Examples of particularly preferred couplers are those described, for example, in U.S. Pat. Nos. 4,124,396, 4,327,173, 4,333,999 and 4,334,011 and Japanese Patent Application (OPI) Nos. 155538/82 and 204545/82, etc.

The light-sensitive material according to the present invention can contain a developing agent, including those described in *Research Disclosure*, Vol. 176, page 29 under the item of "Developing agents".

The light-sensitive material prepared according to the present invention may contain a dye in its photographic emulsion layers or other layers as a filter dye or for various purposes such as prevention of irradiation. Examples of such dyes include those described in *Research Disclosure*, Vol. 176, pages 25 and 26 under the item of "Absorbing and filter dyes".

The light-sensitive material according to the present invention can further contain antistatic agents, plasticizers, matting agents, lubricants, ultraviolet ray absorbing agents, fluorescent brightening agents, air fog preventing agents, etc.

Silver halide emulsion layers and/or other layers are coated on a support by a procedure such as described in *Research Disclosure*, Vol. 176, pages 27 and 28, under the item of "Coating procedures".

Since the compounds according to the present invention have the extremely high bleach accelerating effect, it is possible to attain sufficient silver removal in a short processing time even when a bleaching agent with weak bleaching power is used. Also, the compounds according to the present invention do not adversely affect photographic properties such as color formation, sensitivity and stain properties. Further, the compounds according to the present invention can stably exist in a processing bath for such a long time that problems with control of the bath can be decreased.

The present invention will now be described in more detail with reference to the following examples, however, the present invention is not to be construed as being limited thereto.

#### EXAMPLE 1

On a triacetyl cellulose support provided with a subbing layer were coated in order the emulsion layers and 20 subsidiary layers as described below to prepare a color reversal film.

##### First Layer: Low Sensitive Red-Sensitive Emulsion Layer

25 100 g of a cyan coupler, i.e., 2-(heptafluorobutyramido)-5-[2'-(2",4"-di-tert-amylphenoxy)-butyramido]-phenol was dissolved in 100 ml of tricresyl phosphate and 100 ml of ethyl acetate and stirred at a high speed together with 1 kg of a 10% aqueous gelatin 30 solution to prepare an emulsion. Then, 500 g of the emulsion thus obtained was mixed with 1 kg of a low sensitive red-sensitive silver iodobromide emulsion (containing 70 g of silver and 60 g of gelatin, and having an iodide content of 3 mol%), and the resulting mixture 35 was then coated at a dry thickness of 2 $\mu$  (silver amount: 0.5 g/m<sup>2</sup>).

##### Second Layer: High Sensitive Red-Sensitive Emulsion Layer

40 100 g of a cyan coupler, i.e., 2-(heptafluorobutyramido)-5-[2'-(2",4"-di-tert-amylphenoxy)-butyramido]-phenol was dissolved in 100 ml of tricresyl phosphate and 100 ml of ethyl acetate and stirred at a high speed together with 1 kg of a 10% aqueous gelatin 45 solution to prepare an emulsion. Then, 1 kg of the emulsion thus obtained was mixed with 1 kg of a high sensitive red-sensitive silver iodobromide emulsion (containing 70 g of silver and 60 g of gelatin, and having an iodide content of 3 mol%), and the resulting mixture 50 was then coated at a dry thickness of 2 $\mu$  (silver amount: 0.8 g/m<sup>2</sup>).

##### Third Layer: Intermediate Layer

2,5-Di-tert-octylhydroquinone was dissolved in 100 ml of dibutyl phthalate and 100 ml of ethyl acetate and stirred at a high speed together with 1 kg of a 10% aqueous gelatin solution to prepare an emulsion. Then, 1 kg of the emulsion thus obtained was mixed with 1 kg of a 10% aqueous gelatin solution, and the resulting mixture was coated at a dry thickness of 1 $\mu$ .

##### Fourth Layer: Low Sensitive Green-Sensitive Emulsion Layer

An emulsion was prepared in the same manner as described in the preparation of the emulsion for the first layer except that a magenta coupler, i.e., 1-(2,4,6-trichlorophenyl)-3-[3-(2,4-di-tert-amylphenoxy-acetamido)benzamido]-5-pyrazolone, was used in place

of the cyan coupler. Then, 500 g of the emulsion thus obtained was mixed with 1 kg of a green-sensitive low sensitive silver iodobromide emulsion (containing 70 g of silver and 60 g of gelatin and having an iodine content of 2.5 mol%), and the resulting mixture was coated at a dry thickness of 2.0 $\mu$  (silver amount: 0.7 g/m<sup>2</sup>).

Fifth Layer: High Sensitive Green-Sensitive Emulsion Layer

An emulsion was prepared in the same manner as described in the preparation of the emulsion for the first layer except that a magenta coupler, i.e., 1-(2,4,6-trichlorophenyl)-3-[3-(2,4-di-tert-amylphenoxy-acetamido)benzamido]-5-pyrazolone, was used in place of the cyan coupler. Then, 1 kg of the emulsion thus obtained was mixed with 1 kg of a green-sensitive high sensitive silver iodobromide emulsion (containing 70 g of silver and 60 g of gelatin and having an iodide content of 2.5 mol%), and the resulting mixture was coated at a dry thickness of 2.0 $\mu$  (silver amount: 0.7 g/m<sup>2</sup>).

Sixth Layer: Intermediate Layer

1 kg of the emulsion used in the preparation of the third layer was mixed with 1 kg of a 10% aqueous gelatin solution and coated at a dry thickness of 1 $\mu$ .

Seventh Layer: Yellow Filter Layer

An emulsion containing yellow colloidal silver was coated at a dry thickness of 1 $\mu$ .

Eighth Layer: Low Sensitive Blue-Sensitive Emulsion Layer

An emulsion was prepared in the same manner as described in the preparation of the emulsion for the first layer except that a yellow coupler, i.e.,  $\alpha$ -pivaloyl- $\alpha$ -(1-benzyl-5-ethoxy-3-hydantoinyl)-2-chloro-5-dodecyloxycarbonylacetanilide, was used in place of the cyan coupler. Then, 1 kg of the emulsion thus obtained was mixed with 1 kg of a blue-sensitive low sensitive silver iodobromide emulsion (containing 70 g of silver and 60 g of gelatin and having an iodine content of 2.5 mol%), and the resulting mixture was coated at a dry thickness of 2.0 $\mu$  (silver amount: 0.6 g/m<sup>2</sup>).

Ninth Layer: High Sensitive Blue-Sensitive Emulsion Layer

An emulsion was prepared in the same manner as described in the preparation of the emulsion for the first layer except that a yellow coupler, i.e.,  $\alpha$ -pivaloyl- $\alpha$ -(1-benzyl-5-ethoxy-3-hydantoinyl)-2-chloro-5-dodecyloxycarbonylacetanilide, was used in place of the cyan coupler. Then, 1 kg of the emulsion thus obtained was mixed with 1 kg of a blue-sensitive high sensitive silver iodobromide emulsion (containing 70 g of silver and 60 g of gelatin and having an iodine content of 2.5 mol%), and the resulting mixture was coated at a dry thickness of 2.0 $\mu$  (silver amount: 1.0 g/m<sup>2</sup>).

Tenth Layer: Second Protective Layer

1 kg of the emulsion used in the preparation of the third layer was mixed with 1 kg of a 10% aqueous gelatin solution and coated at a dry thickness of 2.0 $\mu$ .

Eleventh layer: First Protective Layer

A 10% aqueous gelatin solution containing a fine grain emulsion which had not been chemically sensitized (grain size: 0.15 $\mu$ ; 1 mol% silver iodobromide

emulsion) was coated so that the amount of silver coated was 0.3 g/m<sup>2</sup> and the dry thickness was 1 $\mu$ .

The color reversal film thus obtained was subjected to exposure at a proper exposure amount to light having a color temperature of 4,800° K. (adjusted using a filter) from a tungsten light source and then to development processing according to the processing steps described below using various bleaching baths containing the compounds according to the present invention.

| Processing Steps      | Time (min) | Temperature      |
|-----------------------|------------|------------------|
| First Developing Bath | 6          | 38° C.           |
| Washing with Water    | 2          | "                |
| Reversal Bath         | 2          | "                |
| Color Developing Bath | 6          | "                |
| Washing with Water    | 2          | "                |
| Bleaching Bath        | 5          | "                |
| Fixing Bath           | 4          | "                |
| Washing with Water    | 4          | "                |
| Stabilizing Bath      | 1          | Room Temperature |

The composition of each processing solution used in the above described processing was as follows.

|                                                                             |                       |
|-----------------------------------------------------------------------------|-----------------------|
| <u>First Developing Bath</u>                                                |                       |
| Water                                                                       | 700 ml                |
| Sodium Tetrapolyphosphate                                                   | 2 g                   |
| Sodium Sulfite                                                              | 20 g                  |
| Hydroquinone Monosulfonate                                                  | 30 g                  |
| Sodium Carbonate (monohydrate)                                              | 30 g                  |
| 1-Phenyl-4-methyl-4-hydroxymethyl-3-pyrazolidone                            | 2 g                   |
| Potassium Bromide                                                           | 2.5 g                 |
| Potassium Thiocyanate                                                       | 1.2 g                 |
| Potassium Iodide (0.1% solution)                                            | 2 ml                  |
| Water to make                                                               | 1,000 ml<br>(pH 10.1) |
| <u>Reversal Bath</u>                                                        |                       |
| Water                                                                       | 700 ml                |
| 6 Na Salt of Nitrilo-N,N,N-trimethylenephosphonic Acid                      | 3 g                   |
| Stannous Chloride (dihydrate)                                               | 1 g                   |
| p-Aminophenol                                                               | 0.1 g                 |
| Sodium Hydroxide                                                            | 8 g                   |
| Glacial Acetic Acid                                                         | 15 ml                 |
| Water to make                                                               | 1,000 ml              |
| <u>Color Developing Bath</u>                                                |                       |
| Water                                                                       | 700 ml                |
| Sodium Tetrapolyphosphate                                                   | 2 g                   |
| Sodium Sulfite                                                              | 7 g                   |
| Sodium Tertiary Phosphate (12 hydrate)                                      | 36 g                  |
| Potassium Bromide                                                           | 1 g                   |
| Potassium Iodide (0.1% solution)                                            | 90 ml                 |
| Sodium Hydroxide                                                            | 3 g                   |
| Citrazinic Acid                                                             | 1.5 g                 |
| N-Ethyl-N- $\beta$ -methanesulfonamidoethyl-3-methyl-4-aminoaniline Sulfate | 11 g                  |
| Ethylenediamine                                                             | 3 g                   |
| Water to make                                                               | 1,000 ml              |
| <u>Bleaching Bath</u>                                                       |                       |
| Water                                                                       | 800 ml                |
| Sodium Ethylenediaminetetraacetate (dihydrate)                              | 2.0 g                 |
| Iron (III) Ammonium Ethylenediamine-tetraacetate (dihydrate)                | 120.0 g               |
| Potassium Bromide                                                           | 100.0 g               |
| Water to make                                                               | 1,000 ml              |
| <u>Fixing Bath</u>                                                          |                       |
| Water                                                                       | 800 ml                |
| Ammonium Thiosulfate                                                        | 80.0 g                |
| Sodium Sulfite                                                              | 5.0 g                 |
| Sodium Bisulfite                                                            | 5.0 g                 |
| Water to make                                                               | 1,000 ml              |
| <u>Stabilizing Bath</u>                                                     |                       |
| Water                                                                       | 800 ml                |

-continued

|                                                            |          |
|------------------------------------------------------------|----------|
| Formalin (37%)                                             | 5.0 ml   |
| Fuji Driwel (manufactured by<br>Fuji Photo Film Co., Ltd.) | 5.0 ml   |
| Water to make                                              | 1,000 ml |

The silver amount remaining in the maximum density portion of each film sample having been subjected to the development processing as described above was measured according to X-ray fluorometric analysis. The results thus obtained are shown in Table 1 below.

Further, in order to evaluate the stability of the bleach accelerating agents in the bleaching solutions, each bleaching solution containing the bleach accelerating agent as shown in Table 1 below was preserved at 40° C. in a polyethylene bottle for 4 weeks. The same development processing as described above was conducted except for using each bleaching solution thus preserved and the silver amount remaining in the maximum density portion of each sample was measured. The results thus obtained are also shown in Table 1 below.

TABLE 1

| Sample | Bleach Accelerating Agent | Amount Added to Bleaching Bath | Amount of Remaining Silver                |                                                             |
|--------|---------------------------|--------------------------------|-------------------------------------------|-------------------------------------------------------------|
|        |                           |                                | Before Preservation (μg/cm <sup>2</sup> ) | After Preservation (40° C. - 4 weeks) (μg/cm <sup>2</sup> ) |
| 1      | —                         | —                              | 15.3                                      | 15.3                                                        |
| 2      | Compound (2)              | 5 × 10 <sup>-3</sup> mol/l     | 3.5                                       | 3.4                                                         |
| 3      | Compound (3)              | “                              | 3.1                                       | 3.2                                                         |
| 4      | Compound (6)              | “                              | 6.4                                       | 6.6                                                         |
| 5      | Compound (10)             | “                              | 5.5                                       | 5.7                                                         |
| 6      | Compound (11)             | “                              | 3.3                                       | 3.3                                                         |
| 7      | Compound (13)             | “                              | 3.4                                       | 3.5                                                         |
| 8      | Compound (15)             | “                              | 3.6                                       | 3.8                                                         |
| 9      | Compound (16)             | “                              | 3.3                                       | 4.3                                                         |
| 10     | Compound (20)             | “                              | 3.9                                       | 4.4                                                         |
| 11     | Compound (24)             | “                              | 4.7                                       | 4.5                                                         |
| 12     | Compound A                | “                              | 12.6                                      | 15.5                                                        |
| 13     | Compound B                | “                              | 13.4                                      | 15.7                                                        |
| 14     | Compound C                | “                              | 13.7                                      | 15.4                                                        |

Compounds A, B and C used for comparison are as follows:



Compound A

Compound B

Compound C

properties.

## EXAMPLE 2

The same reversal processing as described in Example 1 was conducted except for providing a bleach-fixing solution having the formulation described below in place of both the bleaching solution and the fixing solution, and adding the compound according to the present invention to the bleach-fixing solution (bleach-fixing time: 6 minutes) as shown in Table 2 below. The amount of silver remaining in the film samples was determined in the same manner as described in Example 1. The results thus obtained are shown in Table 2 below.

| Bleach-Fixing Bath                                        |                   |  |
|-----------------------------------------------------------|-------------------|--|
| Iron (III) Ammonium Ethylenediaminetetraacetate Dihydrate | 120.0 g           |  |
| Disodium Ethylenediaminetetraacetate                      | 5.0 g             |  |
| Ammonium Thiosulfate Aqueous Solution (70%)               | 170.0 ml          |  |
| Sodium Sulfite                                            | 10.0 g            |  |
| Water to make                                             | 1,000 ml (pH 6.5) |  |

These compounds are described in Japanese Patent Application (OPI) No. 52534/79.

As is apparent from the results shown in Table 1 above, the bleaching solutions containing the compound according to the present invention have an ex-

65 Further, to each bleach-fixing bath containing the bleach accelerating agent as shown in Table 2 below was added silver bromide in an amount of 16 g/l of the bath and the formation of precipitate was observed with

the naked eye. The results thus obtained are also shown in Table 2 below.

TABLE 2

| Sample | Bleach Accelerating Agent | Amount Added to Bleach-Fixing Bath | Amount of Remaining Silver ( $\mu\text{g}/\text{cm}^2$ ) | Formation of Precipitate |
|--------|---------------------------|------------------------------------|----------------------------------------------------------|--------------------------|
| 15     | Not added                 | —                                  | 110                                                      | Not observed             |
| 16     | Compound (3)              | $1 \times 10^{-2}$ mol/l           | 4.5                                                      | "                        |
| 17     | Compound (6)              | "                                  | 4.7                                                      | "                        |
| 18     | Compound (10)             | "                                  | 5.9                                                      | "                        |
| 19     | Compound (13)             | "                                  | 5.0                                                      | "                        |
| 20     | Compound (18)             | "                                  | 4.8                                                      | "                        |
| 21     | Compound (19)             | "                                  | 6.6                                                      | "                        |
| 22     | Compound (22)             | "                                  | 6.8                                                      | "                        |
| 23     | Compound D                | "                                  | 102                                                      | Observed                 |

Compound D used for comparison is as follows:



Compound D

This compound is described in British Pat. No. 1,138,842.

As is apparent from the results shown in Table 2 above, the removal of silver is also remarkably accelerated when the compound according to the present invention is added to the bleach-fixing bath, and the precipitate was not formed in the bleach-fixing bath when silver ions were present therein. On the contrary, the known Compound D exhibits substantially no bleach accelerating effect and it forms a precipitate in the bleach-fixing bath when silver ions are present therein.

From these results it can be understood that the compounds according to the present invention have excellent properties in that they have extremely large silver removal accelerating function and in that they do not form the precipitate with silver ions when they are added to the bleach-fixing bath.

## EXAMPLE 3

The same reversal processing as described in Example 2 was conducted except for providing a conditioning bath having the formulation described below in place of the washing with water before the bleach-fixing bath, and adding the compound according to the present invention to the conditioning bath as shown in Table 3 below. The amount of silver remaining in the film samples was determined in the same manner as described in Example 1. The results thus obtained are shown in Table 3 below.

| Conditioning Bath                              |          |
|------------------------------------------------|----------|
| Water                                          | 700 ml   |
| Sodium Ethylenediaminetetraacetate (dihydrate) | 8 g      |
| Sodium Sulfite                                 | 12 g     |
| Glacial Acetic Acid                            | 3 ml     |
| Water to make                                  | 1,000 ml |

TABLE 3

| Sample | Bleaching Accelerating Agent | to Conditioning Bath (mol/l) | Amount Added                                             |
|--------|------------------------------|------------------------------|----------------------------------------------------------|
|        |                              |                              | Amount of Remaining Silver ( $\mu\text{g}/\text{cm}^2$ ) |
| 24     | Not Added                    | —                            | 105                                                      |
| 25     | Compound (5)                 | $1 \times 10^{-2}$           | 4.9                                                      |
| 26     | Compound (6)                 | "                            | 4.3                                                      |
| 27     | Compound (13)                | "                            | 6.5                                                      |
| 28     | Compound (15)                | "                            | 4.5                                                      |
| 29     | Compound (18)                | "                            | 5.4                                                      |
| 30     | Compound (19)                | "                            | 6.6                                                      |
| 31     | Compound (22)                | "                            | 5.1                                                      |
| 32     | Compound D                   | "                            | 100                                                      |

Compound D used for comparison was the same compound as used in Example 2.

As is apparent from the results shown in Table 3 above, the removal of silver was accelerated by the addition of the compound according to the present invention to the conditioning bath (i.e., a prebath of the bleach-fixing bath). On the contrary, the known Compound D exhibited substantially no silver removal accelerating effect.

## EXAMPLE 4

On a triacetyl cellulose support were coated layers having the compositions set forth below to prepare a multilayer color photographic light-sensitive material.

## First Layer: Antihalation Layer

A gelatin layer containing black colloidal silver

## Second Layer: Intermediate Layer

A gelatin layer containing a dispersion of 2,5-di-tert-octylhydroquinone

## Third Layer: Low Sensitive Red-Sensitive Emulsion Layer

A silver iodobromide emulsion (iodide content: 5 mol%), silver coated amount: 1.6 g/m<sup>2</sup>

Sensitizing Dye I  $6 \times 10^{-5}$  mol per mol of silver

Sensitizing Dye II  $1.5 \times 10^{-5}$  mol per mol of silver

Coupler EX-1 0.04 mol per mol of silver

Coupler EX-5 0.003 mol per mol of silver

Coupler EX-6 0.0006 mol per mol of silver

## Fourth Layer: High Sensitive Red-Sensitive Emulsion Layer

A silver iodobromide emulsion (iodide content: 10 mol%), silver coated amount: 1.4 g/m<sup>2</sup>

Sensitizing Dye I  $3 \times 10^{-5}$  mol per mol of silver

Sensitizing Dye II  $1.2 \times 10^{-5}$  mol per mol of silver

Coupler EX-2 0.02 mol per mol of silver

Coupler EX-5 0.0016 mol per mol of silver

## Fifth Layer: Intermediate Layer

Same as the second layer

## Sixth Layer: Low Sensitive Green-Sensitive Emulsion Layer

A monodispersed silver iodobromide emulsion (iodide content: 4 mol%), silver coated amount: 1.2 g/m<sup>2</sup>

Sensitizing Dye III  $3 \times 10^{-5}$  mol per mol of silver

Sensitizing Dye IV  $1 \times 10^{-5}$  mol per mol of silver

Coupler EX-4 0.05 mol per mol of silver

Coupler EX-8 0.008 mol per mol of silver

Coupler EX-6 0.0015 mol per mol of silver

**Seventh Layer: High Sensitive Green-Sensitive Emulsion Layer**

A silver iodobromide emulsion (iodide content: 10 mol%), silver coated amount: 1.3 g/m<sup>2</sup>

Sensitizing Dye III  $2.5 \times 10^{-5}$  mol per mol of silver

Sensitizing Dye IV  $0.8 \times 10^{-5}$  mol per mol of silver

Coupler EX-3 0.017 mol per mol of silver

Coupler EX-8 0.003 mol per mol of silver

Coupler EX-10 0.003 mol per mol of silver

**Eighth Layer: Yellow Filter Layer**

A gelatin layer containing yellow colloidal silver and a dispersion of 2,5-di-tert-octylhydroquinone

**Ninth Layer: Low Sensitive Blue-Sensitive Emulsion Layer**

A silver iodobromide emulsion (iodide content: 6 mol%), silver coated amount: 0.7 g/m<sup>2</sup>

Coupler EX-9 0.25 mol per mol of silver

Coupler EX-6 0.015 mol per mol of silver

**Tenth Layer: High Sensitive Blue-Sensitive Emulsion Layer**

A silver iodobromide emulsion (iodide content: 6 mol%), silver coated amount: 0.6 g/m<sup>2</sup>

Coupler EX-9 0.06 mol per mol of silver

**Eleventh layer: First Protective Layer**

A gelatin layer containing silver iodobromide (iodide content: 1 mol%, average particle size: 0.07 $\mu$ ), silver coated amount: 0.5 g/m<sup>2</sup> and a dispersion of Ultraviolet Ray Absorbing Agent UV-1.

**Twelfth Layer: Second Protective Layer**

A gelatin layer containing polymethyl methacrylate particles (having a diameter of about 1.5 $\mu$ ).

Gelatin Hardener H-1 and sodium di(2-ethylhexyl)sulfosuccinate as a surface active agent were incorporated into each of the layers in addition to the above described components.

15 The compounds used for preparing the sample were as follows:

Sensitizing Dye I: Pyridinium salt of anhydro-5,5'-dichloro-3,3'-di( $\gamma$ -sulfopropyl)-9-ethylthiacarbocyanine hydroxide

20 Sensitizing Dye II: Triethylamine salt of anhydro-9-ethyl-3,3'-di( $\gamma$ -sulfopropyl)-4,5,4',5'-dibenzo-thiacarbocyanine hydroxide

Sensitizing Dye III: Sodium salt of anhydro-9-ethyl-5,5'-dichloro-3,3'-di( $\gamma$ -sulfopropyl)oxacarbocyanine

Sensitizing Dye IV: Sodium salt of anhydro-5,6,5',6'-tetrachloro-1,1'-diethyl-3,3'-di[ $\beta$ -[ $\beta$ -( $\gamma$ -sulfo-propoxy)ethoxy]ethyl]imidazolocarbocyanine hydroxide

Couplers



EX-1



EX-2



EX-3



EX-4

$n/m + m' = 1$ ,  $m/m' = 1$  (ratio by weight)  
molecular weight: about 40,000



EX-5

-continued  
Couplers



|    | Processing Steps   | Time           |
|----|--------------------|----------------|
| 45 | Color Development  | 3 min & 15 sec |
|    | Bleaching          | 4 min & 20 sec |
|    | Fixing             | 4 min & 20 sec |
|    | Washing with Water | 3 min & 15 sec |
|    | Stabilizing        | 30 sec         |

## GELATIN HARDENER H-1



## ULTRAVIOLET RAY ABSORBING AGENT UV-1



x/y = 7/3 (ratio by weight)

The resulting photographic material was subjected to exposure to light in an exposure amount of 25 CMS using a tungsten light source and a filter to adjust the color temperature to 4,800° K. and then to development processing at 38° C. according to the following processing steps.

|    |                                                           |                       |
|----|-----------------------------------------------------------|-----------------------|
| 55 | Color Developing Solution                                 |                       |
|    | Trisodium Nitrilotriacetate                               | 1.9 g                 |
|    | Sodium Sulfite                                            | 4.0 g                 |
|    | Potassium Carbonate                                       | 30.0 g                |
|    | Potassium Bromide                                         | 1.4 g                 |
|    | Potassium Iodide                                          | 1.3 mg                |
| 60 | Hydroxylamine Sulfate                                     | 2.4 g                 |
|    | 4-(N-Ethyl-N-β-hydroxyethylamino)-2-methylaniline Sulfate | 4.5 g                 |
|    | Water to make                                             | 1,000 ml<br>(pH 10.0) |
| 65 | Bleaching Solution                                        |                       |
|    | Iron (III) Ammonium Ethylenediaminetetraacetate           | 80.0 g                |
|    | Disodium Ethylenediaminetetraacetate                      | 8.0 g                 |
|    | Ammonium Bromide                                          | 120.0 g               |
|    | Compound According to the Present                         | Amount shown          |

-continued

|                                                |                      |
|------------------------------------------------|----------------------|
| Invention (shown in Table 4)                   | in Table 4           |
| Water to make                                  | 1,000 ml<br>(pH 6.0) |
| <u>Fixing Solution</u>                         |                      |
| Sodium Tetrapolyphosphate                      | 2.0 g                |
| Sodium Sulfite                                 | 4.0 g                |
| Ammonium Thiosulfate Aqueous Solution<br>(70%) | 175.0 ml             |
| Sodium Bisulfite                               | 4.6 g                |
| Water to make                                  | 1,000 ml<br>(pH 6.6) |
| <u>Stabilizing Solution</u>                    |                      |
| Formalin (40%)                                 | 8.0 ml               |
| Water to make                                  | 1,000 ml             |

The above described development processing was also conducted as above using the same bleaching bath as described above but not containing the compound according to the present invention.

Each film sample having been subjected to development processing in the above described manner was subjected to X-ray fluorometric analysis to determine the silver amount remaining in the maximum density portion of the sample. The results thus obtained are shown in Table 4 below.

Further, in the same manner as described in Example 1, each bleaching bath as shown in Table 4 below was subjected to the thermal preservation at 40° C. in a polyethylene bottle for 4 weeks, the same development processing as described above was conducted except for using each bleaching bath thus preserved and the silver amount remaining in the maximum density portion of each sample was measured. The results thus obtained are also shown in Table 4 below.

TABLE 4

| Sam-<br>ple | Bleach<br>Agent | Amount<br>Added to<br>Bleaching | Amount of Remaining Silver  |                                            |
|-------------|-----------------|---------------------------------|-----------------------------|--------------------------------------------|
|             |                 |                                 | Before<br>Preserva-<br>tion | After<br>Preservation<br>(40° C., 4 weeks) |
| 33          | Not Added       | —                               | 11.5                        | 11.6                                       |
| 34          | Compound (3)    | $5 \times 10^{-3}$              | 2.0                         | 2.1                                        |
| 35          | Compound (4)    | "                               | 3.1                         | 3.3                                        |
| 36          | Compound (8)    | "                               | 4.3                         | 4.1                                        |
| 37          | Compound (12)   | "                               | 4.5                         | 4.6                                        |
| 38          | Compound (15)   | "                               | 3.4                         | 3.2                                        |
| 39          | Compound (17)   | "                               | 3.0                         | 3.3                                        |
| 40          | Compound (18)   | "                               | 4.7                         | 4.7                                        |
| 41          | Compound (20)   | "                               | 5.1                         | 5.0                                        |
| 42          | Compound (22)   | "                               | 5.4                         | 5.5                                        |
| 43          | Compound (24)   | "                               | 4.6                         | 4.6                                        |
| 44          | Compound A      | "                               | 10.2                        | 11.8                                       |
| 45          | Compound C      | "                               | 10.8                        | 11.7                                       |
| 46          | Compound D      | "                               | 11.0                        | 11.7                                       |

Compounds A, C and D used for comparison are the same compounds as used in Examples 1 and 2.

As is apparent from the results shown in Table 4 above, the compounds according to the present invention also remarkably accelerated removal of silver in the processing of the color negative photographic light-sensitive material in comparison with the known Compounds A, C and D and the compounds according to the present invention had good stability in the bleaching solution. On the contrary, the known Compounds A, C and D were poor in the stability in the bleaching solution and had substantially no silver removal accelerating effect.

### EXAMPLE 5

The same processing as described in Example 4 was conducted except for providing a bleach-fixing bath having the same formulation as described in Example 2 in place of the bleaching bath and the fixing bath, and adding the compound according to the present invention (shown in Table 5 below) to the bleach-fixing solution (bleach-fixing time was 4 minutes). The silver amount remaining in the film samples was determined in the same manner as described in Example 4. The results thus obtained are shown in Table 5 below.

TABLE 5

| Sample | Bleach Accelerating Agent | Amount Added to Bleach-Fixing Bath (mol/l) | Amount of Remaining Silver ( $\mu\text{g}/\text{cm}^2$ ) |
|--------|---------------------------|--------------------------------------------|----------------------------------------------------------|
| 47     | Not Added                 | —                                          | 60                                                       |
| 48     | Compound (2)              | $1 \times 10^{-2}$                         | 3.5                                                      |
| 49     | Compound (3)              | "                                          | 3.0                                                      |
| 50     | Compound (6)              | "                                          | 5.2                                                      |
| 51     | Compound (7)              | "                                          | 3.4                                                      |
| 52     | Compound (9)              | "                                          | 3.6                                                      |
| 53     | Compound (15)             | "                                          | 4.2                                                      |
| 54     | Compound (18)             | "                                          | 3.8                                                      |
| 55     | Compound (20)             | "                                          | 5.1                                                      |
| 56     | Compound (22)             | "                                          | 4.4                                                      |
| 57     | Compound A                | "                                          | 55                                                       |
| 58     | Compound B                | "                                          | 56                                                       |
| 59     | Compound D                | "                                          | 58                                                       |

Compounds A, B and D used for comparison are the same compounds as used in Examples 1 and 2.

As is apparent from the results shown in Table 5 above, the use of the compound according to the present invention in the bleach-fixing bath remarkably accelerated removal of silver in the processing of the color negative photographic light-sensitive material in comparison with the known Compounds A, B and D.

While the invention has been described in detail and with reference to specific embodiments thereof, it will be apparent to one skilled in the art that various changes and modifications can be made therein without departing from the spirit and scope thereof.

What is claimed is:

1. A method for processing a color photographic light-sensitive material by subjecting an exposed silver halide color photographic light-sensitive material to color development, then to bleaching and fixing or then to bleach-fixing, which method comprises using a ferric ion complex salt as a bleaching agent in the bleaching or bleach-fixing and incorporating at least one compound represented by general formula (I) described below or a tautomer thereof:



wherein X represents N or C—R; R, R<sup>1</sup>, R<sup>2</sup> and R<sup>3</sup>, which may be the same or different, each represents a hydrogen atom, a halogen atom, an amino group, a hydroxyl group, a carboxyl group, a sulfo group or an alkyl group; R<sup>4</sup> and R<sup>5</sup>, which may be the same or different, each represents a hydrogen atom, an alkyl group or an acyl group or R<sup>4</sup> and R<sup>5</sup> may be bonded to

each other to form a ring, provided that both  $R^4$  and  $R^5$  do not represent a hydrogen atom at the same time; and  $n$  represents an integer of 0 to 5, in a bleaching bath, bleach-fixing bath or in a prebath of the bleach-fixing bath.

2. A method for processing a color photographic light-sensitive material as claimed in claim 1, wherein the alkyl group represented by  $R$ ,  $R^1$ ,  $R^2$ ,  $R^3$ ,  $R^4$  or  $R^5$  is a substituted or unsubstituted alkyl group having from 1 to 5 carbon atoms in the alkyl moiety.

3. A method for processing a color photographic light-sensitive material as claimed in claim 2, wherein a substituent for the substituted alkyl group for  $R$ ,  $R^1$ ,  $R^2$ ,  $R^3$ ,  $R^4$  or  $R^5$  is one member selected from the group consisting of a halogen atom, a hydroxyl group, an alkoxy group, a sulfonyl group, a carbamoyl group, a sulfamoyl group, a carboxyl group, a sulfo group, an amino group, an amido group, and a sulfonamido group.

4. A method for processing a color photographic light-sensitive material as claimed in claim 1, wherein the ring formed by bonding  $R^4$  and  $R^5$  is one member selected from the group consisting of a pyrrole ring, an imidazole ring, a pyrazole ring, a piperidine ring and a morpholine ring.

5. A method for processing a color photographic light-sensitive material as claimed in claim 1, wherein the acyl group represented by  $R^4$  or  $R^5$  is an acyl group having 3 or less carbon atoms.

6. A method for processing a color photographic light-sensitive material as claimed in claim 1, wherein the acyl group represented by  $R^4$  or  $R^5$  is an acetyl group.

7. A method for processing a color photographic light-sensitive material as claimed in claim 1, wherein the compound represented by general formula (I) is incorporated into the bleaching bath.

8. A method for processing a color photographic light-sensitive material as claimed in claim 1, wherein the compound represented by general formula (I) is incorporated into the bleach-fixing bath.

9. A method for processing a color photographic light-sensitive material as claimed in claim 1, wherein the compound represented by general formula (I) is incorporated into the prebath of the bleach-fixing bath.

10. A method for processing a color photographic light-sensitive material as claimed in claim 1, wherein the amount of the compound represented by general formula (I) in the bleaching bath, the bleach-fixing bath or the prebath of the bleach-fixing bath is from about

$1 \times 10^{-5}$  to about 1 mol per liter of a processing solution.

11. A method for processing a color photographic light-sensitive material as claimed in claim 9, wherein the prebath is an aqueous solution containing the compound represented by general formula (I) and having a pH of about 9 or less.

12. A method for processing a color photographic light-sensitive material as claimed in claim 1, wherein the ferric ion complex salt is a complex of ferric ion and a chelating agent.

13. A method for processing a color photographic light-sensitive material as claimed in claim 12, wherein the chelating agent is an aminopolycarboxylic acid, an aminopolyphosphonic acid or a salt thereof.

14. A method for processing a color photographic light-sensitive material as claimed in claim 13, wherein the salt of an aminopolycarboxylic acid or an aminopolyphosphonic acid is an alkali metal salt, an ammonium salt or a water-soluble amine salt.

15. A method for processing a color photographic light-sensitive material as claimed in claim 1, wherein the bleaching bath contains a re-halogenating agent.

16. A method for processing a color photographic light-sensitive material as claimed in claim 1, wherein the amount of the ferric ion complex salt is from about 0.1 to about 2 mols per liter of the bleaching solution.

17. A method for processing a color photographic light-sensitive material as claimed in claim 1, wherein the bleach-fixing bath contains a ferric ion complex salt and a fixing agent.

18. A method for processing a color photographic light-sensitive material as claimed in claim 17, wherein the amount of the ferric ion complex salt is from 0.1 to 2 mols and the amount of the fixing agent is from 0.2 to 4 mols, per liter of the bleach-fixing solution.

19. A method for processing a color photographic light-sensitive material as claimed in claim 1, wherein the silver halide color photographic light-sensitive material is a multilayer color photographic light-sensitive material.

20. A method for processing a color photographic light-sensitive material as claimed in claim 19, wherein the multilayer color photographic light-sensitive material is a color reversal photographic light-sensitive material or a color negative photographic light-sensitive material.

\* \* \* \* \*